

## UNITED STATES PATENT OFFICE.

CHARLES R. SHORT, OF DAYTON, OHIO, ASSIGNOR TO GENERAL MOTORS RESEARCH CORPORATION, OF DAYTON, OHIO, A CORPORATION OF DELAWARE.

## METHOD OF MAKING WROUGHT-METAL ARTICLES.

No Drawing.

Application filed July 2, 1925. Serial No. 41,114.

- This invention relates to the manufacture of metallic objects by a combination of casting and forging, or other similar metal-working steps. By "metal-working" is meant such operations as impart to metal the characteristics of so-called "wrought" metal, that is, operations that deform the metal or cause it to flow more or less, such as rolling, hammer or press forging, drawing, extruding or the like.
- It is an object of the invention to produce metallic articles having the desirable properties of wrought metal, without subjecting the metal to the extremes of distortion and molecular flow incident to the forging of articles to final form from ingot, billet or bar. In the usual practice of making wrought metal articles, the extent of flow is considerable and the direction of flow is not as a rule controllable. It follows that where very considerable changes of size and form are produced by forging, the metal flows in various directions and some parts flow more than others. In consequence the articles are apt to be weaker in some parts than in others. The weaknesses due to excessive flow are more apt to occur in some kinds of metal than in others. It is particularly desirable not to work excessively, for example, aluminum and certain other alloys.
- A further defect due to excessive working by pressure is the piping or "radishing" flaw that frequently develops in the interior of wrought metal articles, which is wholly concealed.
- According to this invention, when it is desired to produce any given metal article, a mold is made, which is approximately a counterpart of the desired article, but is somewhat larger, and a blank is cast in this mold by pouring into it molten metal of the kind desired. The oversize blank thus formed may now be reduced in order to form the finished article by any process of working suited to the particular blank and article. The blank may, for example, be compressed between forging or rolling dies of a size and contour to reduce the blank to final size. The working pressure thus applied will cause some flow of metal, sufficient to close up interstices, such as blow holes, and fill small cavities resulting from failure of the metal to completely fill or flow to all parts of the mold. It will endow the article with the desirable qualities of wrought metal and impart a finish to the metal superior to that incident to unfinished castings.
- The casting operation may be performed preferably in chill or die molds. These molds may be of iron, copper or other metal suitable for die molds. Metallic or die molds conduct heat from the casting quickly and, therefore, cause the casting to set quickly and enable it to be removed quickly. Quick setting and removal of the casting reduces the likelihood of deformation or flaws in the casting due to shrinking in the molds. By using metal molds which cool the casting rapidly, certain metallic compositions with a suitable proportion of silicon may be used as the casting metal, whereby to obtain a more ductile or malleable product than could be obtained by casting in a sand mold.
- The method under consideration has been found of great utility in making articles of certain light alloys such as magnesium and aluminum alloys. For example, an aluminum alloy, high in silicon may be first cast in an oversize metal mold that is an approximate counterpart of the article to be made, removed therefrom soon after it has set and before it has lost so much heat as to cause it to shrink to any great extent, and may then be compacted to final size between forging dies.
- The silicon content should be sufficient to produce an alloy that is "hot short" within the narrowest possible range of temperature, and may be cast to advantage within chilled molds.
- After removal from the mold the blank may be forged while still hot from the casting operation, provided the casting is of such composition as will stand forging at that temperature. Castings made from compositions may be forged while they are still hot from the casting operation. Others may be forged cold. Still others, among them the aluminum alloy referred to, may require for best results a reheating, while some may require a heat-treatment after forging.
- The special utility of the described method applied to manufacture of articles from light alloys or homogeneous mixtures of metals, lies in the fact that it avoids certain defects of prior processes. In these mixtures or alloys, as in many others in which the different ingredients have rather widely separated melting points, there is a tendency for the ingredients to separate when a casting is set-

- ting or freezing from a molten state. The higher melting point ingredients, freezing first, squeeze out the lower melting point ingredients. As a result, when the alloy hardens it is weak in spots owing to the segregation of particular ingredients; so, castings of these alloys are of uncertain and variable strength. Consequently the practice has hitherto obtained of making articles of such alloys, by a process of working them by forging or other pressure, from ingot, billet or bar, to final shape, the products of the exclusive working process being subject to the other defects already mentioned.
- 15 By casting, according to this method, alloys of the type mentioned in metal molds, the casting cools so quickly that there is insufficient time for the ingredients to segregate materially. By reason of the rapid setting of the casting, it may be removed from the mold before sufficient shrinkage occurs to tear or weaken the metal in the mold. This is a very important circumstance in casting articles, which, like connecting rods, have 20 separated enlargements connected by a part of smaller cross-section. In castings of this form the enlarged portions, being anchored in the mold, are apt to tear partly away from the smaller portions during shrinkage if left 25 in the mold, thus developing a serious flaw. By the method of this invention, flaws of the kind described are avoided, and superior castings obtained.
- If the casting, made and removed as described, is then worked under pressure all over so as to slightly reduce its cross-sectional area, without excessive flow, the article may be perfected in finish, the metal compacted, interior holes closed and external 30 cavities filled by slight flow of the metal. Thus the described casting has imparted to it the desirable qualities of wrought metal free of the defects incident to manufacture wholly by pressure working.
- 45 By this method, metal articles of rather slight malleability, which cannot be successfully wrought entirely by forging, may be manufactured and will be found to possess to a degree the qualities of wrought metal 40 articles without their defects.
- In making, for example, a light alloy connecting rod by this method, a die or metallic mold will be made which is approximately a counterpart of the finished article desired but slightly larger. The alloy will then be poured in a molten condition into the die or mold. As soon as the blank thus cast, has set, the die or mold will be opened and the cast blank removed. If the heat in the blank 55 is above that at which the material of the blank is hot-short it should immediately be forged to size, as in forging dies which are a counterpart in size of the desired finished article. Otherwise, the blank may be reheated to 60 the requisite temperature and then wrought 65 to size. A heat-treatment may be given the finished article after forging, if the properties of the particular alloy used render it desirable.
- In casting connecting rods, it is desirable 70 to provide suitable cores or bosses within the mold to provide the necessary recesses for the crank and wrist pin in order to avoid piping, and to thereafter forge the casting with metallic plugs inserted in the recesses. 75
- While the form of embodiment of the invention as herein disclosed, constitutes a preferred form, it is to be understood that other forms might be adopted, all coming within the scope of the claims which follow. 80
- What is claimed is as follows:
1. A method of making metallic articles, which consists in casting a blank in a chill mold that is approximately a counterpart of but somewhat larger than the desired article, removing the cast blank and reducing it to final size by working it under pressure. 85
  2. The method of making metallic articles, which consists in casting a blank in a mold that is approximately a counterpart of but 90 slightly larger than the desired article, removing the cast blank, and reducing it to final size by working it under pressure while still hot from the casting operation.
  3. A method of making metallic articles, 95 which consists in casting a blank in a chill mold that is approximately a counterpart of but somewhat larger than the desired article, removing the cast blank from the mold before it has cooled enough to shrink materially, 100 and reducing said blank to final size by working it under pressure.
  4. The method of making articles from alloys containing metallic constituents of substantially different melting points, said constituents tending to separate from a molten mixture thereof when cooling, which consists in pouring molten alloy metal of the kind described into a chill mold that is approximately a counterpart of but somewhat larger 105 than the desired article, said mold being of sufficient conductivity to cause the cast blank to set before separation can take place, removing the cast blank and reducing it to final size by working it under pressure. 110
  5. The method of making articles from alloys containing metallic constituents of substantially different melting points, said constituents tending to separate from a molten mixture thereof when cooling, which consists in pouring molten alloy metal of the kind described into a chill mold that is approximately a counterpart of but somewhat larger 115 than the desired article, said mold being of sufficient conductivity to cause the cast blank to set before separation can take place, removing the cast blank from the mold, and reducing it to final size by compressing it in forging dies which are a counterpart of the desired article. 120
  6. The method of making articles from alloys containing metallic constituents of substantially different melting points, said constituents tending to separate from a molten mixture thereof when cooling, which consists in pouring molten alloy metal of the kind described into a chill mold that is approximately a counterpart of but somewhat larger 125 than the desired article, said mold being of sufficient conductivity to cause the cast blank to set before separation can take place, removing the cast blank from the mold, and reducing it to final size by compressing it in forging dies which are a counterpart of the desired article. 130

6. The method of making articles from alloys containing metallic constituents of substantially different melting points, said constituents tending to separate from a molten mixture thereof when cooling, which consists in pouring molten alloy metal of the kind described into a chill mold that is approximately a counterpart of but somewhat larger than the desired article, said mold being of sufficient conductivity to cause the cast blank to set before separation can take place, removing the cast blank after it has set and before it has cooled enough to shrink materially, and reducing it to final size by working it under pressure.
7. The method of making articles from alloys containing metallic constituents of substantially different melting points, said constituents tending to separate from a molten mixture thereof when cooling, which consists in pouring molten alloy metal of the kind described into a chill mold that is approximately a counterpart of but somewhat larger than the desired article, said mold being of sufficient conductivity to cause the cast blank to set before separation can take place, removing the cast blank from the mold, and reducing it to final size by working it under pressure at a temperature above that at which the metal of the casting is hot-short.
8. The method of making articles from an alloy of aluminum containing silicon, which consists in pouring said alloy in molten condition into a chill mold that is approximately a counterpart of but somewhat larger than the desired article, removing the cast blank from the mold after it has set and before it has cooled enough to shrink materially, and reducing it to final size by working it under pressure.
9. The method of making articles from an alloy of aluminum containing silicon, which consists in pouring said alloy in molten condition into a chill mold that is approximately a counterpart of but somewhat larger than the desired article, removing the cast blank from the mold after it has set and before it has cooled enough to shrink materially, and reducing it to final size by working it under pressure.
10. The method of making articles from an alloy of aluminum containing silicon, which consists in pouring said alloy in molten condition into a chill mold that is approximately a counterpart of but somewhat larger than the desired article, removing the cast blank from the mold, and reducing it to final size by working it under pressure at a temperature above that at which the metal of the casting is hot-short.
11. The method of making articles from an alloy of aluminum containing silicon, which consists in pouring said alloy in a molten condition into a chill mold that is approximately a counterpart of but somewhat larger than the desired article, removing the cast blank from the mold after it has set and before it has cooled enough to shrink materially, and reducing it to final size by compressing it in forging dies which are a counterpart of the desired article.

In testimony whereof I hereunto affix my signature.

CHARLES R. SHORT.